

101

CROSS REFERENCE

C. A. PFANSTIEHL.  
PROCESS FOR CLEANING CONTACT POINTS.  
APPLICATION FILED JULY 11, 1914.  
1,304,803.

Patented May 27, 1919.



Witnesses  
Albin C. Allerg  
Robert F. Bracke

Inventor  
Carl A. Pfanstiehl  
By *John C. Williams*  
Attorney.

# UNITED STATES PATENT OFFICE.

CARL A. PFANSTIEHL, OF WAUKEGAN, ILLINOIS, ASSIGNOR, BY MESNE ASSIGNMENTS, TO PFANSTIEHL COMPANY, INC., OF NORTH CHICAGO, ILLINOIS, A CORPORATION OF NEW YORK.

## PROCESS FOR CLEANING CONTACT-POINTS.

1,304,803.

Specification of Letters Patent.

Patented May 27, 1919.

Application filed July 11, 1914. Serial No. 850,350.

*To all whom it may concern:*

Be it known that I, CARL A. PFANSTIEHL, a citizen of the United States, residing in Waukegan, in the county of Lake and State 5 of Illinois, have invented certain new and useful Improvements in Processes for Cleaning Contact-Points, of which the following is a full, clear, concise, and exact description, reference being had to the accompanying 10 drawings, forming a part of this specification.

My invention relates to a process for cleaning contact points, more particularly contact points having contact faces or surfaces of tungsten and the object of my invention is to remove from the tungsten contact point the metal which accumulates thereon during the process of mounting the tungsten contact point as will be more fully 20 hereinafter explained.

Metallic tungsten is one of the group of so-called rare metals. It fuses at extremely high temperatures and does not readily oxidize or corrode in ordinary atmosphere. It 25 is extremely hard and therefore can not be cut or worked with ordinary tools. Its properties are such as to make it admirably adapted for electrical contact points of electrical switching mechanisms of various 30 types but the high cost of the material itself together with the difficulties in working it into shape for use has in the past practically prevented its application as a material from which to make electrical contact points.

In constructing an electrical contact point of the class mentioned I preferably cut from a tungsten rod of the proper diameter a disk of tungsten of suitable thickness. This disk of tungsten is subsequently fused or welded 40 upon a base metal backing, such for example as steel or iron, by interposing an extremely thin disk or film of copper between the tungsten disk and its associated base metal backing and then subjecting the 45 tungsten disk, backing and intermediate copper film or disk to the extremely high temperature produced within a suitable electric furnace. While this invention is not particularly concerned with the mechanism 50 for cutting the tungsten disk from the end of a rod or with the details of the electric furnace, it may be well at this point to say that during the fusing or welding operation an atmosphere of hydrogen is preferably maintained within the electric furnace to pre-

vent oxidation of the base metal backing and copper disk or film.

I find that during the fusing or welding operation just mentioned a considerable portion of the copper interposed between the tungsten disk and its associated base metal 60 backing will flow out over the cylindrical surface of the tungsten disk. It is necessary in order to provide a satisfactory contact point to remove the copper from the surface 65 of the tungsten disk. It is the object of my present invention to remove this copper without resorting to a process of grinding or polishing which would be quite expensive and generally unsatisfactory. My invention 70 is fully set forth in the following description in which reference is made to the accompanying drawings in which—

Figure 1 illustrates a tungsten disk, a base metal backing, and intermediate copper disk 75 or film ready to be placed in the electric furnace, and

Fig. 2 is a view of the same parts after the fusing or welding operation has been completed and after the excess copper has 80 been removed from the tungsten disk by my improved process hereinafter described.

Referring first to Fig. 1 at A I have illustrated a tungsten disk and at B I have shown a base metal backing provided with an integral shank C. It will be understood that the shank C may be passed through a suitable aperture in a contact-spring or switch-lever and there riveted to retain the backing B and parts carried thereby in operative position. Interposed between the tungsten disk A and the backing B is an extremely thin disk or film D, preferably of copper. In practice the copper disk D is preferably 1-1/2/1000 or 2/1000 of an inch in thickness. 95

After the several parts have been assembled as illustrated in Fig. 1 they are placed in a suitable electric furnace and the temperature within the furnace is raised to a point considerably above the fusing point 100 of the copper. The tungsten disk A is thus fused or welded to the base metal backing B. I find that during the fusing or welding operation a considerable portion of the copper interposed between the disk A and the 105 backing B flows out of the space between the backing and disk and covers the cylindrical surface of the tungsten disk A. In practice I find that the film of copper remaining between the tungsten disk A and the backing 110

B after the fusing or welding operation has a thickness of not greater than substantially 1/1000 of an inch, that portion of the copper flowing from between the tungsten disk 5 A and the backing B covering the cylindrical surface of the contact. As before stated it is necessary that this excess copper be removed to provide a satisfactory contact point.

10 In accordance with my present invention I provide a shallow dish, preferably of earthen-ware, and within this shallow earthen-ware dish I place a layer of welded contact points. I then place this dish upon 15 a plate kept cool by means of running water and then cover the contact points with concentrated nitric acid mixed with a small quantity of heavy paraffin oil. The paraffin oil which is very thick and sluggish has a 20 very high surface tension. Before adding the solution of concentrated nitric acid and paraffin oil to the contact points it is advisable to stir the solution inasmuch as the oil and nitric acid tend somewhat to separate 25 when permitted to stand indefinitely. As will presently be made apparent it is desirable that the nitric acid when added to the contact points have a very high surface tension. If the acid is kept extremely cool 30 by means of running water its surface tension is materially increased. An inert thick substance such as heavy paraffin oil materially increases the surface tension of the nitric acid.

35 I find it desirable to leave the contact points in the mixture of nitric acid and paraffin oil for approximately ten or fifteen minutes, although no harm is done if the points are left in this mixture for a considerably longer period. The reason for this 40 is that the mixture of nitric acid and paraffin oil is extremely viscous and has a high surface tension. The surface tension is so great that after the acid has eaten slightly 45 into the copper between the tungsten disk and the base metal backing there will be no circulation of acid within this space. The acid which comes into contact with the copper disk between the backing and the tungsten disk becomes spent and no acid works 50 its way into the space mentioned to continue the chemical disintegration of the copper.

In Fig. 2 I have illustrated how the acid eats into the copper disk but a slight distance. It will be understood that if it were 55 not for the high surface tension of the acid to the action of which the contact points are subjected the acid would eat its way rapidly into the space between the tungsten disk and its base metal support and thus detach 60 the tungsten from its support.

After the contact points have been permitted to remain in the acid solution for approximately ten or fifteen minutes the solution is poured off and the contacts are 65 dipped in a weak caustic solution, such for example as caustic soda or caustic potash. The points are then rinsed in clear water and dried. I find that if the points are washed in water before being rinsed in the 70 caustic solution there is a tendency to acidulate the water and the weak solution of nitric acid having an extremely low surface tension will work its way into the space between the tungsten disk and its associated 75 support and thus dissolve the copper film which is depended upon for the weld.

Having thus described my invention what I claim as new and desire to secure by Letters Patent is,

80

1. The process of cleaning contacts of the class described which consists in subjecting the contacts to the attack of a viscous acid solution, rinsing the contacts in a weak caustic solution and rinsing the contacts in 85 water.

2. The process of cleaning contacts of the class described which consists in subjecting the contacts to the attack of a viscous acid solution and then rinsing the contacts in a 90 weak caustic solution.

3. The process of cleaning contacts of the class described which consists in subjecting the contacts to the action of a solution of concentrated nitric acid and paraffin oil and 95 then rinsing the contacts thus treated in a weak caustic solution.

In witness whereof I hereunto subscribe my name this 8th day of July, A. D. 1914.

CARL A. PFANSTIEHL.

Witnesses:

ALBIN C. AHLBERG,  
MARY A. COOK.